

[54] PROCESS FOR MANUFACTURING STEEL

[75] Inventor: Aldo Ramacciotti, Rome, Italy

[73] Assignee: Centro Sperimentale Metallurgico  
S.p.A., Rome, Italy

[22] Filed: May 6, 1971

[21] Appl. No.: 140,962

|           |        |                     |       |
|-----------|--------|---------------------|-------|
| 979,605   | 1/1965 | Great Britain ..... | 75/60 |
| 991,579   | 5/1965 | Great Britain ..... | 75/60 |
| 1,110,054 | 4/1968 | Great Britain ..... | 75/60 |

Primary Examiner—Hyland Bizot

Assistant Examiner—Peter D. Rosenberg

Attorney, Agent, or Firm—Young &amp; Thompson

## [30] Foreign Application Priority Data

May 22, 1970 Italy ..... 50894/70

[52] U.S. Cl. .... 75/60, 75/61

[51] Int. Cl. .... C21c 5/32

[58] Field of Search ..... 75/61, 60, 59, 51, 52, 46,  
75/11

## [56] References Cited

## UNITED STATES PATENTS

|           |         |                       |         |
|-----------|---------|-----------------------|---------|
| 3,689,250 | 9/1972  | Roeder .....          | 75/11   |
| 2,828,516 | 4/1958  | Black et al.....      | 266/37  |
| 2,962,277 | 11/1960 | Morrill.....          | 75/60   |
| 3,015,554 | 1/1962  | Rummel.....           | 75/60   |
| 3,672,869 | 6/1972  | Niehaus .....         | 75/60   |
| 2,862,811 | 12/1958 | Eketorp et al.....    | 75/60   |
| 2,959,479 | 11/1960 | Graef .....           | 75/60   |
| 3,271,128 | 9/1966  | Tartaron .....        | 75/60   |
| 2,978,318 | 4/1961  | Kalling et al.....    | 75/60 X |
| 3,313,619 | 4/1967  | Decamps .....         | 75/60   |
| 3,034,885 | 5/1962  | Hardt.....            | 75/52   |
| 2,977,217 | 3/1961  | Graef et al.....      | 75/60   |
| 3,251,681 | 5/1966  | Wakamatsu et al ..... | 75/61   |
| 3,401,034 | 9/1968  | Moore .....           | 75/61   |

## FOREIGN PATENTS OR APPLICATIONS

943,267 12/1963 Great Britain ..... 75/60

## [57] ABSTRACT

Process for manufacturing steel, particularly special and alloyed, in a vessel revolving around its vertical axis, furnished with means for varying sharply its velocity or reversing the sense of rotation, said vessel being internally lined with basic or acid refractory, the steelmaking being carried out by downwardly blowing oxydizing gases, in particular technically pure oxygen, over the melt consisting of liquid pig iron, iron or steel scarp and/or iron in pigs, flux and possibly iron ore, said melt being dynamically curved by the rotation; in which process the oxygen required for the refining, or other oxydizing or inert gases are blown downwardly, these being called primary jet, and other oxygen and/or other oxydizing gases, called secondary jet, are blown down in order to burn up to 90 percent of CO formed during the refining actions and form CO<sub>2</sub> inside the vessel, including the metallic melt is directly overheated by the heat developed by said combustion of CO, without using other fuels, being the refractory lining of the vessel protected against the action of the heat as well as of the slag during the refining.

1 Claim, No Drawings

## PROCESS FOR MANUFACTURING STEEL

The present invention relates to an improved process for manufacturing steel. More particularly, the object of this invention is a process wherein the charge material (liquid pig iron, with scrap, slag, flux and if the case may be also iron ore) is contained in a vertical symmetrical vessel, revolving at a suitable speed and sense about its vertical axis and will be refined by blowing onto its surface, by means of suitable devices, oxidizing refining gas, particularly technically pure oxygen.

As it is known from the prior art, the making of non common and alloyed steel requires the recourse to relatively long processes, the use of particularly selected charges (steelmaking in electric furnace) or of cumbersome, space requiring and expensive plants having a low yield (Martin-Siemens furnaces).

Other processes at present used, like those known under the names of LD (or BOF) and LD-AC allow the treatment times to be remarkably shortened with respect to the previous art and particularly with respect to the conventional Bessemer and Thomas converters, and require relatively simple plants; however by these processes steels of a normal quality are produced, and high amounts of scraps cannot be used. In order to obviate this drawback it has been proposed to pre-heat the scrap within or outside the converter, but this operation requires pre-heating plants which are rather expensive and complicated, or the use of silicon carbide and/or calcium carbide, with a consequent increase of the manufacturing cost.

Another technical proposed solution consists in increasing the temperature inside the converter by burning therein suitable fuels, particularly the carbon monoxide which is formed during the refining process.

However, in a stationary converter, most of the refractory is exposed to the intense heat generated by this combustion of CO, and thus it will be worn in a very short time.

Thereby the need derives of getting rid of the heat absorbed in a refractory in a useful way; so was invented the furnace revolving about a horizontal or subhorizontal axis, wherein the area of the refractory lining which is not submerged is over-heated by the combustion of carbon oxide and then, due to its revolution, it contacts the metal bath and delivers thereto part of the absorbed heat. This type of process, although rather spread, shows severe drawbacks due to wear of the refractory as the whole surface thereof is exposed in sequential times, to the damages caused by heat, to the attack of the slag and to the erosion due to the friction between the metal bath, which is almost stationary, and the lining which is revolving. These reasons render the average life of the refractory lining of these furnaces somewhat lower than that of a conventional LD converter.

Several attempts have been made in order to diminish the damage of the refractory, but none of them reached the aimed purpose. For instance the French Pat. No. 1,207,464 describes a converter revolving at high speed about its vertical axis, provided with spout hole through its bottom and further provided with a lance blowing on the bath surface, dynamically disposed against the vertical walls of the converter, a refining gas, through a set of nozzles distributed along a generatrix of the lance itself located parallel to the bath. The jets of the so blown gas will cause an intense

rabbling of the metal with the slag, and further hit an ever new surface, thus reducing the local temperature and the formation of "red smokes."

On the ground of tests carried out with revolving converters, it has been noted that if one part of the bottom of the converter is left uncovered and exposed to the direct action of the heat and, in an annular zone also to the slag attack, as in fact it occurs in said French Patent, the other advantages as aforesaid will be reduced to a determinant amount; in fact the part of refractory left uncovered will undergo a quick physical degradation, so that after a very reduced number of heats, the work must be discontinued and the refractory lining must be restored. Also the high speeds of revolution up to 500 rev./min., as disclosed in said French Patent do not appear to be the most suitable for an industrial-type converter. In said Patent, also, no word is spent for the possibility of over-heating the bath by supply of a heat different from that generated by the refining reactions.

It is evident, therefore, that up to now no process has been actuated conciliating the need of using installations which are capable of operating for a long time requiring no relining, with the need of making high grade steels in very short times and at a lower cost.

According to the present invention it is possible to overcome the above cited drawbacks concerning the refractory consumption, by providing a process whereby it is possible to make special steels in times comparable to those of the LD process, but with a greater production capacity at parity of internal volume of the converter, and therefore at a lower cost.

The process forming the object of the present invention consists in refining a charge including liquid pig iron, steel scrap and/or iron in pigs, flux and possibly iron ore and/or other cooling material by blowing one or more streams of refining oxygen or other oxidizing gas, mixed, if the case may be, with inert gas (argon, nitrogen and the like) in a proportion variable up to the double of the rate of oxygen and/or of the oxidizing gas, called primary jet in the following disclosure, on the surface of said bath, suitably dynamically curved, while simultaneously a determined amount of oxygen and other oxidizing gas, called secondary jet, is blown in order to burn to CO<sub>2</sub>, inside the converter, the carbon monoxide developed during the refining reactions, wherein the blowing of said primary jet and of said secondary jet ensures a quick development of the refining reactions and therefore an effective overheating of the bath, the refractory lining being protected against the heat action during the refining. This is possible insofar as the revolution of the converter, and therefore of the molten bath, determines a distribution of a part of the molten mass of the bath against almost the entire vertical wall of the converter, screening it against the intense heat generated during said combustion action, the balance remaining to protect the bottom. Furthermore, according to the present invention, this rise of the bath along the walls of the converter is utilized in order so to increase the amount of the charge, so that the ratio: total converter inner volume/weight of the charge, is equal at the utmost to 0.4 m<sup>3</sup>/t versus a ratio of about 0.8 to 1 m<sup>3</sup>/t which can be obtained in a vertical stationary converter. It is to be noted that this increase of charge does not prevent the refining times from being kept within the limits of a conventional LD process; in fact due to revolution, the thickness of the

bath will be at any point suitable for a quick and effective refining. The speed of revolution of the converter appears to be rather critical to the purposes of both the metallurgical process and the protection of the refractory. The thickness of the bath, in fact, must be such as to prevent the primary jet from reaching the lining of the converter and at same time must be not so great as to promote the generation of "dead zones" little interested or not interested to the refining reactions. It has been found that preferably the revolution speed must be such as to allow the formation of a paraboloid the height of which stands in a relation with the internal diameter of the converter according to a ratio comprised between 0.7 and 1.5.

Furthermore, to avoid the wear of the refractory due to the friction between the latter and the bath, according to the present invention, the speed of revolution of the converter must be established in relation to the dimensions of the converter itself, so that at the rated speed, the peripheral speeds of the basic or acid refractory and of the metal bath, at the separating surfaces thereof will be equal, avoiding, as aforesaid, that wear which hindered a large diffusion of those processes, for instance the Kaldo process, where said relative movements exist.

Another feature of the present invention, connected to the primary blowing, consists in that the slag is kept apart from the basic or acid lining so that said slag cannot attack the lining. In fact the slag which is lighter than the liquid metal, will locate on the surface of the paraboloid generated by the rotation of the bath and tends to rise, heaping near the upper end of said paraboloid. This fact would involve the double drawback of wearing quickly the refractory zone concerned with the heaping of the slag, and of leaving the bath at the point or points of impact of the oxygen and/or the oxidizing gas, free from slag, slowing down the refining process. These drawbacks will be overcome, according to the present invention, by directing the primary jet so as to maintain utmost of the slag at the apex of the paraboloid, the remaining part being located on the bath in the form of a thin layer and/or of foam.

It has been found that this purpose and together that of an optimum development of the refining reactions, can be attained according to this invention, by directing the primary jet so as to hit the bath at a characteristic position, variable according to the form and capacity of the vessel; particularly it has been found that for the industrial converters, the impact point of the primary jet onto the surface of the paraboloid must be at a distance from the axis of the converter, measured on the radius of the cross section of the converter at that point, comprised between 10 percent and 40 percent of the value of the internal diameter of the converter itself.

Due to this particular blowing, certain streams will be formed on the surface of the paraboloid and above said impact point, said streams being directed towards the impact point itself and hindering the upwards movement of the slag due to centrifugal force; under this impact point the strength of the jet itself keeps the slag gathered at the apex of the paraboloid, the speed of rotation being such as to ensure that each point of the paraboloid come to be located under the primary jet before the slag had been capable of climbing remarkably beyond said impact point. Thus an effective rabbling of

the slag with the molten bath will be obtained with a consequent improvement of the refining.

According to the present invention, furthermore, the blowing of the primary jet is carried out by means of a lance with a vertical single nozzle which is eccentrically located and adjustable both vertically and horizontally, the eccentricity of which is comprised between 10 percent and 40 percent of the value of the internal diameter of the converter, said lance being so located that its head will be at a distance from the impact point comprised between 20 percent and 65 percent of the value of the internal diameter of the converter.

In a further embodiment of the process according to this invention, the blowing is carried out through a lance located at the centre, along the vertical axis of the converter; in this case said lance is provided with one or more nozzles, downwards directed with their axes inclined with respect to the axis of the lance itself through an angle from 15° to 45°. This lance is vertically adjustable and its distance measured along the axis of the nozzles, from said nozzles to the impact point of said jets on the surface of the bath, equals a value from 18 percent to 65 percent of the value of the internal diameter of the converter.

Another feature of the present invention consists in that the heat developed by the combustion of CO to CO<sub>2</sub> is absorbed directly by the metal bath, rotated by means known per se, as disclosed in the first part of this specification. In fact according to this invention, an amount up to 90 percent of said CO will be effectively burnt, utilizing the combustion heat in order to melt amounts of scrap from 20 percent to more than 50 percent of the total charge and/or corresponding amounts of pig iron in pigs and/or iron ores, with no need of pre-heating or of the addition of other fuel. According to the amount of cold charge it is possible to utilize said combustion heat also for overheating the metal bath, so as to be in a position as to carry out, at the end of the refining operation, further metallurgical operations in order to obtain a high grade final product.

The blowing of the secondary jet is embodied according to the present invention so that this secondary jet hit directly neither the surface of the metal bath nor that of the refractory; particularly, said secondary jet is delivered through nozzles the diameter of which varies from 1/50 to 1/150 of the distance measured along the axis of the nozzles themselves, from said nozzles to the molten bath.

If the primary jet is blown by an eccentric lance, the blowing of the secondary jet can be obtained by means of a second lance vertically and horizontally adjustable, the eccentricity of said second lance varying from nil to the value of the eccentricity of the primary lance, said second lance having one or more nozzles and being introduced into the converter so that said nozzles will be at a depth, measured from the mouth of the vessel, from 10 percent to 40 percent of the value of the internal diameter of the converter.

If the blowing of the primary jet is effected by means of a lance located along the axis of the converter, the secondary jet will be blown by auxiliary nozzles, suitably located along the circumference of the head of the lance spaced apart from the end less than two diameters of the lance, or along the circumference of the lance body. In this second case the auxiliary nozzles are downwards turned and are inclined with respect to the axis of the lance through an angle from 10° to 30°; their

position inside the converter is so selected as to establish their distance from the plane of the mouth at a value from 10 percent to 40 percent of the internal diameter of the converter itself. If the main lance is located along the axis of the converter the blowing of the secondary jet can also be made of a second lance provided with one or more nozzles, located eccentrically and horizontally or vertically adjustable, with an eccentricity variable from 10 percent to 40 percent of the value of the internal diameter of the converter. This second lance is introduced into the converter so that said nozzles will be located at a variable depth measured from the mouth of the converter; the maximum effect will be reached at a depth from 10 percent to 40 percent of the internal diameter of the converter. The rate of this secondary jet can vary from 40 percent to 100 percent of the value of the rate of the primary jet, said secondary rate being adjustable, independently from that of the primary jet, during the process, from zero to the optimum value.

The over-heating caused by the combustion of CO is such as to render useless the addition of slag fluidizing substances, and furthermore it is capable of allowing, at the end of refining, subsequent operations of slag replacement, of purifying and of alloying: thus, in a short while and with no subsequent supplies of heat a high grade product will be obtained, which could not be obtained by processes having an equal duration, and comparable to, or higher than that which can be obtained in far longer times with the electric furance. Moreover, the aforesaid fact that part of the surface of the bath is covered only by a thin layer of slag will render quicker and more effective the overheating of the bath itself.

The process according to this invention results to be particularly flexible; it can be utilized not only in those plants where scarce amounts of liquid pig iron are available, but also in plants where the liquid pig iron contains high amounts of sulphur and phosphorus as well as of other oxidizable impurities. Also in this case the process according to this invention is capable of bringing the refining to values which cannot be attained by any other process, in correspondingly short times.

In order to better illustrate the advantages of the present invention, hereinafter there are: a Table (Table 1) summarizing the data of certain heats effected, some examples of process and a Table (Table 2) showing the refractory consumption, wherein by way of example some average attained results are shown together with some preferred types of process, according to the present invention.

Table 1 shows the data of certain heats, selected in the groups of heats carried out for testing the various type of blowing.

Column 1 shows the data of one of the first heats carried out to ascertain the validity of the process, and wherein only primary oxygen has been blown.

Columns 2, 3, 4 and 5 show the data of heats effected by blowing also secondary oxygen. Two lances have been used with variable eccentricity and penetration inside the converter.

Columns 6, 7 and 8 show the data of casting effected by blowing also secondary oxygen and utilizing a single lance capable of delivering, from different nozzles, primary and secondary oxygen.

In the columns 1, 2, 3, 5 and 7 possible additions of iron alloys were subsequently effected in the ladder.

In the castings 4, 6 and 8 the Fe-Si has been added in the converter.

#### EXAMPLE 1

5 This example relates to the heat reported in Table 1 under No. 5. In this heat the effectiveness of the process has been tested under the standpoint of the refining as well as of the final yield. The sequence of the operations has been as follows:

10 1. Charging part of the lime (about two-fifths of the total), then scrap, liquid pig iron, and lastly other two-fifths of lime, in the order;

2. starting the converter rotating;

3. lowering the main lance and low-pressure blowing;

15 4. stabilizing simultaneously the speed of revolution at the rated value;

5. mixing for de-phosphorizing; replacing the slag;

6. putting into operation the main lance and the main

20  $O_2$  blowing has reached its rated value;

7. starting of the decarburization and addition of the last amount of lime;

8. positioning of the secondary lance and starting blowing the secondary  $O_2$ ;

25 9. blowing of secondary  $O_2$  at its rated value;

10. removing the secondary lance; rating the secondary  $O_2$  to nil;

11. discontinuing the main  $O_2$  blowing;

12. simultaneously removing the primary lance and

30 starting stopping the converter;

13. short rabbling;

14. converter stopped; tilting of the converter, temperature measurement and bath and slag sampling;

35 15. inclining of the converter and tapping.

During the test there was a slight "slopping" during the first minutes of blowing.

The primary oxygen was blown by an eccentric lance with one nozzle and the secondary oxygen was blown by a lance also eccentric and with two nozzles having

40 a 32 mm diameter. The percent ratio, between the rate of secondary  $O_2$ , and the rate of the primary  $O_2$  was equal to 100.

As is shown in the Table, the ratio between the final sulphur and the initial sulphur is 0.33 and the ratio between the final phosphorus and the initial phosphorus is about 0.062.

The oxygen and nitrogen content of the steel resulted to be less than 0.001 percent. The iron yield was 93.6 percent.

50 50 A rabbling cycle consists in starting the converter and causing it to reach the rated speed, then stopping the converter, and subsequently starting it in opposite sense, and finally stopping it again.

#### EXAMPLE 2

This example relates to the heat reported in Table 1, under No. 6.

This heat, one of the first heat effected with a single lance and delivery of primary and secondary  $O_2$ , was directed to ascertain the capacity of desulphurization. To this purpose of liquid pig iron with a very high sulphur content and a little amount of scrap has been charged. The operative sequence has been identical to that shown in Example 1, apart from the fact that the rabbling and the slag replacement according to point 5 have not been carried out, and after the operation 12, the following operations have been carried out:

13. stopping the converter; tilting, temperature measurement and slag and steel sampling;  
 14. putting the converter in vertical position, slagging with two rabbling cycles;  
 15. adding deoxidizing agent and lime;  
 16. two rabbling cycles;  
 17. tilting the converter; temperature measurement slag and steel sampling;  
 18. tapping.

The single lance, in axial position, had two nozzles for delivering primary O<sub>2</sub>, and six nozzles for delivering secondary O<sub>2</sub>. Said secondary nozzles were located in the converter at a depth corresponding to 20 percent of the diameter of the converter itself, and their diameter was 0.6 percent of the distance from said nozzles to the metal bath.

The final sulphur/initial sulphur ratio was 0.089, while no de-phosphorization operation being carried out the ratio of the final phosphorus to initial phosphorus was 0.33.

- 5 The oxygen content of the final steel was 0.0091 and the nitrogen content was 0.010.

Owing to the relatively small capacity of the used converter, and due to a remarkable slopping and of the various slag replacing operations, the iron yield has been 88.5 percent.

The Table 2 shows the refractory consumption after 50 non continuous heats.

- 10 15 As the refractory was a dolomite ramming, its consumption resulted lower than that usually obtained.

TABLE 1

| Heat No.                                                           | 1      | 2      | 3      | 4     | 5      | 6     | 7      | 8     |
|--------------------------------------------------------------------|--------|--------|--------|-------|--------|-------|--------|-------|
| Percent composition of the charge:                                 |        |        |        |       |        |       |        |       |
| Liquid pig iron.....                                               | 83     | 74     | 65     | 83    | 71     | 83    | 56     | 80    |
| Scrap.....                                                         | 13     | 22     | 30     | 13    | 25     | 13    | 40     | 14    |
| Lime.....                                                          | 4      | 4      | 5      | 4     | 4      | 4     | 4      | 6     |
| Percent composition of the liquid pig iron:                        |        |        |        |       |        |       |        |       |
| C.....                                                             | 3.6    | 3.5    | 3.6    | 3.6   | 3.6    | 3.32  | 3.6    | 3.4   |
| Si.....                                                            | 0.49   | 0.75   | 1.01   | 0.56  | 0.62   | 0.62  | 0.48   | 0.84  |
| Mn.....                                                            | 0.64   | 0.85   | 0.84   | 0.87  | 0.72   | 0.64  | 0.61   | 0.70  |
| P.....                                                             | 0.10   | 0.11   | 0.15   | 0.13  | 0.16   | 0.16  | 0.09   | 0.11  |
| S.....                                                             | 0.032  | 0.057  | 0.054  | 0.045 | 0.079  | 0.112 | 0.063  | 0.033 |
| T°C.....                                                           | 1405   | 1370   | 1364   | 1370  | 1366   | 1370  | 1373   | 1371  |
| Primary blowing characteristics:                                   |        |        |        |       |        |       |        |       |
| Eccentricity/conv. diam. (percent) .....                           | 30     | 20     | 15     | 20    | 25     | 25    | 40     | 60    |
| Height/conv. diam. (percent).....                                  | 25     | 40     | 20     | 25    | 25     | 25    |        |       |
| Secondary blowing characteristics:                                 |        |        |        |       |        |       |        |       |
| Eccentricity/conv. diam. (percent).....                            | 0      | 10     | 20     | 20    | 20     | 20    |        |       |
| Depth/conv. diam. (percent).....                                   | 50     | 15     | 20     | 30    | 20     | 25    | 15     |       |
| No. of nozzles.....                                                | 4      | 2      | 2      | 2     | 6      | 4     | 6      |       |
| Nozzles diam./bath dist. (percent).....                            | 0.6    | 3.2    | 3.2    | 3.2   | 0.4    | 0.6   | 0.8    |       |
| Sec. rate O <sub>2</sub> /prim. rate O <sub>2</sub> (percent)..... | 61     | 100    | 100    | 100   | 100    | 77    | 100    |       |
| Ratio of comb. burnt CO/produced CO (percent).....                 | 41     | 54     | 64     | 52    | 77     | 43    | 38     |       |
| O <sub>2</sub> total consumption Nm <sup>3</sup> /t steel.....     | 51     | 44     | 55     | 58    | 49     | 53    | 46     | 43    |
| Blowing duration min.....                                          | 19     | 15     | 18     | 15    | 22     | 15    | 14     | 18    |
| Slagging and subsequent rabblings:                                 |        |        |        |       |        |       |        |       |
| No. of cycles.....                                                 |        |        | 3      | 6     | .....  | 4     | .....  | 4     |
| Blow. duration/work duration (percent).....                        |        |        | 100    | 53.6  | .....  | 52    | .....  | 52    |
| Final composition of steel when tapped (percent):                  |        |        |        |       |        |       |        |       |
| C.....                                                             | 0.14   | 0.16   | 0.08   | 0.40  | 0.16   | 0.37  | 0.09   | 0.50  |
| Mn.....                                                            | 0.28   | 0.29   | 0.09   | 0.19  | 0.14   | 0.35  | 0.13   | 0.22  |
| Si.....                                                            | traces | traces | traces | 0.25  | traces | 0.17  | traces | 0.26  |
| P.....                                                             | 0.022  | 0.021  | 0.005  | 0.029 | 0.010  | 0.053 | 0.009  | 0.034 |
| S.....                                                             | 0.022  | 0.035  | 0.016  | 0.004 | 0.026  | 0.01  | 0.026  | 0.026 |
| O.....                                                             |        |        | 0.0065 |       | 0.0091 |       |        |       |
| N <sup>2</sup> .....                                               |        |        | 0.010  |       | 0.0080 |       |        |       |
| T°C.....                                                           | 1660   | 1625   | 1590   | 1632  | 1615   | 1621  | 1620   | 1646  |
| Iron yield.....                                                    | 94.8   | 95.2   | 93.4   | 94.0  | 93.6   | 88.5  | 92.9   | 94.7  |
| Slag characteristics at the end point:                             |        |        |        |       |        |       |        |       |
| Total Fe.....                                                      | 17.2   | 12.5   | 26.1   | 20.0  | 21.6   | 10.5  | 23.1   | 14.2  |
| Basicity index.....                                                | 3.4    | 3.5    | 5.2    | 5.0   | 4.7    | 2.6   | 4.8    | 3.3   |

TABLE 2

Distance from mouth/total useful height of the converter, (percent)

| 0                                                         | 7  | 11 | 14 | 17 | 21 | 25 | 29 | 32 | 36 | 39 | 43 | 46 ÷ 65 | 68 ÷ 74 | 77 ÷ 100 |
|-----------------------------------------------------------|----|----|----|----|----|----|----|----|----|----|----|---------|---------|----------|
| Thickness of eroded refractory/total thickness, (percent) |    |    |    |    |    |    |    |    |    |    |    |         |         |          |
| 32.5                                                      | 25 | 22 | 25 | 24 | 20 | 20 | 18 | 15 | 10 | 10 | 1  | 0       | 1       | 0        |

Having thus described the present invention what is claimed is:

1. In a process for manufacturing steel, comprising establishing in a vessel having a refractory lining and having a vertical axis a quantity of molten ferrous metal under a blanket of slag, rotating the vessel about said vertical axis to impart to the molten ferrous metal a substantially concave paraboloidal surface about said axis, and blowing against said surface a jet of gas containing oxygen; the improvement comprising directing said jet of gas against said surface a distance from said

axis in a direction to urge said slag toward said axis and away from said refractory lining, said distance being 10 to 40 percent of the inner diameter of the vessel, the speed of rotation of the vessel being such that said paraboloidal surface has a height whose ratio to the internal diameter of the vessel is between 0.7 and 1.5, and the filling ratio of the vessel, expressed as the ratio between the total inner volume of the vessel in cubic meters and the charge weight in metric tons, being below 10 0.4.

\* \* \* \* \*